

Nov. 11, 1958

D. J. WEST ET AL. 2,860,079  
HEAT TREATING PROCESS FOR A 2% Fe 2% Cr 2%  
Mo TITANIUM BASE ALLOY  
Filed May 25, 1955



INVENTORS.  
DONALD J. WEST  
RICHARD A. BAUGHMAN  
BY

*John F. Cullen*

ATTORNEY—

# United States Patent Office

2,860,079

Patented Nov. 11, 1958

1

2,860,079

## HEAT TREATING PROCESS FOR A 2% Fe 2% Cr 2% Mo TITANIUM BASE ALLOY

Donald John West and Richard Augustus Baughman, Cincinnati, Ohio, assignors to General Electric Company, a corporation of New York

Application May 25, 1955, Serial No. 511,115

4 Claims. (Cl. 148—13)

This invention relates to a process for heat treating titanium and in particular to a process for heat treating a particular type of titanium alloy in order to make it ductile.

Compressor wheels of a turbojet engine are a critical part of the engine and are subjected to high migratory stresses when rotating at high velocity. Also, large stress concentrations take place when the turbojet engine undergoes sudden bursts of thrust during transient operation. The points of stress concentrations take place in areas where there is a tendency for the stresses to build up. If the material undergoing these stress concentrations has ductility, the material can undergo plastic deformation at the point of stress concentration and relieve the stress. If the stress concentration continues to build up and is not relieved, it can result in the form of an initial fracture which will later destroy the part and perhaps destroy the engine. This problem becomes particularly critical during the high speeds of a jet engine at which time the temperature and velocity of rotating parts is also exceedingly high, so that any initial fracture will be seriously aggravated and undoubtedly do a lot of damage to the engine. Since titanium alloy has a good strength weight ratio, the use of compressor wheels made from titanium alloys is very desirable in order to achieve considerable weight savings in the engine. However, one of the undesirable features of titanium is that it tends to remain brittle mainly because of the impurities contained in the alloy itself. Therefore, the ductility necessary to meet the specification requirements is a problem confronting the entire titanium industry. It is therefore a general object of this invention to provide a process for heat treating titanium articles to give them the necessary ductility required to comply with the specifications.

In forging titanium, the article previously has been formed high in the beta and alpha plus beta range to give the material the necessary ductility. However, in forming articles in the beta and alpha plus beta range, it has been difficult to consistently obtain the properties required by specifications because of the lack of data on heat treating cycles to produce a material ductile and stable enough to allow the manufacture of titanium alloy articles. Therefore large amounts of titanium articles are rejected and scrapped. Since titanium is a very expensive material, scrapping is very expensive. In general, approximately 50% of the compressor wheels made of titanium and heat treated to the previous processes fail to meet the specification requirement for ductility and are rejected. It is therefore another general object of this invention to provide a process for heat treating titanium articles to consistently meet the required ductility.

A further object of this invention is to provide a process for heat treating a titanium alloy in the beta and alpha plus beta phases without permitting the formation of fine alpha structure in order to obtain improved ductility.

2

It is another object of this invention to provide a heat treating process for an alloy in which the material is heated to a temperature in the beta field to form a beta structure and then transformed isothermally at a temperature in the alpha plus beta phase to produce a ductile material.

These and other objects will become more apparent when read in the light of the accompanying specification, taken in connection with the attached drawing. The scope of our invention will be pointed out in the appended claims.

The drawing is a time-temperature-transformation diagram for the titanium alloy which includes about 2% iron, 2% chromium and 2% molybdenum.

In general, the invention may be practiced by heating an alloy comprising about 2% iron, about 2% chromium, about 2% molybdenum, the balance essentially titanium to a temperature exceeding the alpha plus beta transformation temperature, maintaining the alloy at this temperature for a period of time, and then transforming the alloy isothermally to an alpha plus beta structure at a lower temperature.

In order to heat treat titanium alloy articles made of approximately 2% of iron, 2% of chromium, 2% of molybdenum and the rest titanium and its impurities, so as to have the necessary ductility to meet the required specifications, the first step is betatizing the article by heating to 1650 F. into the area marked "beta" in the drawing. Betatizing is a term used in connection with heat treating a material in the beta field. It is noted that the oxygen can influence the transformation temperature as well as the contaminations found in the material. These factors could raise the beta temperature. It is desirable however to heat the material in the beta field while staying as low in the beta field as possible. The primary reason for doing this is to form a beta structure with a minimum amount of alpha phase before transforming back into the alpha plus beta field as shown in the drawing. To get rid of all of the alpha, it is necessary to stay at this low temperature in the beta field, otherwise fine alpha may remain and will result in accompanying low ductility of the material. Therefore, by staying at the low temperature in the beta field, the fine alpha will be eliminated to a substantial extent so that the material in general contains beta before transforming back to an alpha plus beta structure at the lower temperature. In betatizing a material it is noted that the time in general is not too critical so long as the material is maintained at this temperature sufficiently long to be stabilized at that temperature.

The next step in the process is the isothermal heat treating portion in which the material is cooled down to 1325° F. This can be done by transferring to another furnace which is already at the 1325° F. temperature or staying in the furnace and cooling it down to 1325° F. Either method of cooling has been found satisfactory so long as the material is not permitted to cool down below 1325° F. At 1325° F. coarse alpha, shown by the shaded portion in the drawing, is allowed to form. It is noted that the 1325° F. temperature is very critical in this instance in that dropping below the 1325° F. temperature, fine alpha will form. It is this fine alpha that forms in the structural composition of this material when in the alpha plus beta phase that causes brittleness when cooling down to room temperature. Also, it is noted that if the material is held at a higher temperature than 1325° F., less alpha forms in reaching equilibrium conditions, and more of it stays beta so that upon subsequent cooling the additional beta transforms to fine alpha and causes brittleness. The time at 1325° F. for the best results is found to be 13 hours. This time is critical and it is necessary to maintain an isothermal

condition until equilibrium between alpha and beta phases is established. The minimum time at 1325° F. is approximately 11 hours, depending on the material itself so long as equilibrium is reached and coarse alpha is formed.

After stabilizing the material at 1325° F. the material is then furnace cooled to 1200° F. This step is necessary since after cooling from 1325° F. additional alpha may be formed. In other words, at any lower temperature, more alpha is present at equilibrium conditions than at 1200° F. or 1325° F. The beta to alpha transformation is a time-temperature phenomenon. In order to have alpha and beta in equilibrium at a given temperature, sufficient time for transformation must be allowed. Also, the lower the temperature, the slower the reaction. Long times at 1200° F. are therefore necessary to allow the alpha and beta phases to reach equilibrium in the alpha plus beta region shown in the drawing and prevent the formation of an unstable beta phase upon subsequent cooling to room temperature. If insufficient time is allowed at 1200° F. and unstable beta forms, then a fine precipitate or fine alpha will form from the unstable beta during subsequent engine operation, causing loss of ductility.

It is therefore necessary to cool the material to 1200° F. and stabilize this material by transforming it into the alpha plus beta phase at that temperature for 24 hours. Although the material can cool down to room temperature from the 1325° F. and then be heated to 1200° F., it has been found that cooling to 1200° F. instead of dropping down to room temperature, tends to keep scaling of the titanium down to a minimum.

The last step of the process is cooling the material to room temperature by taking the article out of the furnace. It is noted that cooling down to room temperature by taking the article out of the furnace is much better than furnace cooling since brittleness again results when furnace cooling is employed thereby making the ductility of the material low.

The following table which is the summary of tests conducted on six different heats of material compares the physical properties of the titanium base alloy containing about 2% iron, about 2% chromium and about 2% molybdenum before and after our novel heat treatment. The marked increase in ductility is especially to be noted:

|                                 | Before  | After   |
|---------------------------------|---------|---------|
| Tensile Strength (p. s. i.)     | 139,600 | 132,100 |
| 0.2% Yield Strength (p. s. i.)  | 131,600 | 123,200 |
| 0.02% Yield Strength (p. s. i.) | 119,100 | 113,300 |
| Percent Elongation              | 12.0    | 21.0    |
| Percent Reduction in Area       | 17.0    | 31.0    |

In order to show the stability of this particular titanium alloy after our novel heat treatment process, a series of compressor wheel rings were aged for up to about 1000 hours. The following table summarizes the results of aging showing uniform increased ductility:

| Aging Temp. (° F.) | Hours at Temp. | Ductility after Heat Treatment (Percent Elongation) |
|--------------------|----------------|-----------------------------------------------------|
| 500                | 0              | 16                                                  |
| 500                | 100            | 16                                                  |
| 500                | 295.5          | 16                                                  |
| 500                | 500            | 16                                                  |
| 500                | 703            | 16                                                  |
| 500                | 967            | 16                                                  |

Additional test results showing the increase in ductility resulting from the use of our novel heat treatment is

shown by the following table which summarizes a series of tests performed on compressor discs:

| 5  | Sample Series | Before Heat Treatment |                           | After Heat Treatment |                           |
|----|---------------|-----------------------|---------------------------|----------------------|---------------------------|
|    |               | Percent Elongation    | Percent Reduction In Area | Percent Elongation   | Percent Reduction In Area |
| 10 | M 139         | 11                    | 14                        | 21                   | 30                        |
|    | R 122         | 8                     | 12                        | 15                   | 15                        |
|    | L 130         | 5                     | 7                         | 15                   | 15                        |

In summary therefore, a step treatment for heat treating titanium is provided to result in a titanium alloy of improved ductility in which the material is heated to its lowest point in the beta range and held at this temperature until the material becomes all beta. The next step is furnace cooling to 1325° F. and holding the temperature until as much coarse alpha that is going to form at that temperature takes place. The material is then furnace cooled again to 1200° F. and held for a sufficient length of time to produce the alpha plus beta structure. This stabilizes the material and prevents fine alpha from being precipitated. The elimination of fine alpha prevents brittleness and eventual age hardening during engine operation. The last step is cooling the material in air to room temperature.

It is noted that the heat treatment temperatures of 1325° F. and 1200° F. must be maintained for sufficient periods of time to produce ductility and provide a stable alpha plus beta microstructure.

The above example of the invention has been given by way of illustration and is not intended as a limitation of the invention. The time and temperatures given can vary within narrow limits according to the characteristics of the material, such variations being intended to be included within the spirit and scope of this invention.

40 What we claim as new and desire to secure by Letters Patent of the United States is:

1. The process of heat treating a titanium alloy including about 2% iron, about 2% chromium and about 2% molybdenum comprising heating to approximately 1650° F. to form the beta phase, maintaining this temperature until such time as the material becomes stabilized, furnace cooling to 1325° F. and maintaining this temperature for approximately 13 hours permitting coarse alpha phase in equilibrium with beta phase to form without permitting fine alpha to form, cooling to 1200° F. and maintaining this temperature for 24 hours to prevent fine alpha from forming, and air cooling to room temperature.

2. In a heat treating process for a titanium alloy including about 2% iron, about 2% chromium and about 2% molybdenum, heating to the lowest temperature in the beta range and holding at this temperature until all of the material becomes beta, cooling to about 1325° F. and holding this temperature for approximately 13 hours to permit as much alpha as is going to form to take place, furnace cooling to 1200° F. to stabilize the material to prevent age embrittling, air cooling this material to room temperature.

3. In a process for heating titanium alloy consisting of 2% iron, 2% chromium, 2% molybdenum and the rest titanium and its impurities, heating the material to the beta range to form as much beta as possible, cooling the material to the alpha plus beta range without permitting fine alpha to form, annealing at 1200° F. and maintaining this temperature long enough to stabilize the material to prevent age embrittling, and air cooling the material to room temperature.

4. The process of heat treating a titanium alloy including about 2% iron, about 2% chromium and about 2% molybdenum comprising heating at approximately 1650°

F. for about one hour, furnace cooling to about 1325° F., maintaining 1325° F. for approximately 13 hours to permit coarse alpha phase to form in equilibrium with beta phase without permitting fine alpha to form, air cooling to room temperature, heating to 1200° F. and maintaining this temperature for about 24 hours to prevent fine alpha from forming and then air cooling to room temperature.

## References Cited in the file of this patent

## UNITED STATES PATENTS

2,596,485 Jaffee et al. May 13, 1952  
5 2,754,203 Vordahl July 10, 1956

## OTHER REFERENCES

Atlas of Isothermal Transformations, U. S. Steel, pages 6-26, 1951.